

## UNITED STATES PATENT OFFICE

2,507,082

## CORE MATERIALS

Jim E. Allison, Elmhurst, Ill., assignor to The Quaker Oats Company, Chicago, Ill., a corporation of New Jersey

No Drawing. Application June 21, 1946,  
Serial No. 678,352

2 Claims. (Cl. 22—188)

1

The present invention relates to core materials, and more particularly to cereal core binders employed in their production.

My invention is concerned with the production of a corn product core binder. In the past various corn products have been proposed by the prior art as foundry core binders. For example, a first type of prior art product is produced by sending a heavy slurry of mill starch from a corn wet processing plant over the hot surfaces of internally heated rolls. The contact of the mill starch slurry with the heated surfaces causes the gelatinization of the starch and the formation of a flaked product which is then ground to a fine powder. A second type of prior art product is made by moistening degeminated corn and subjecting the moistened product to a heated roll surface whereby the starch in the degeminated ground corn is gelatinized and whereby the whole product is flaked. The flaked gelatinized product is then ground to a fine powder.

I have found that ground degeminated corn can, when properly processed, be made into an efficient core binder having qualities superior to that obtained with corn product fractions of the prior art. Heretofore in making foundry cores for use in the production of castings, it has been the practice to mix core sand with a variety of dry or liquid binders, namely: various corn product fractions, pulverized cereals, pulverized foundry pitch, rosin or casein, sulphite pulp waste liquor, molasses, or various oils such as linseed, soybean or other vegetable oils. The mixture of sand and binder is then moistened with sufficient water so that it can be inserted into core boxes of various shapes and sizes corresponding to the shape and sizes of cavities it is desired to produce by means of the cores.

When the corebox is removed, the grains of sand must be bound together by the binder so as to permit handling in an approved manner and transferring to an oven. In the oven the cores are baked to expel the water, drive off volatile constituents and give a core capable of withstanding the pressure encountered in casting operations. In casting, the heat of the molten metal burns out the binder, the gases from which vent through the core and molds, leaving the core in a friable form or as loosely held sand readily removable from the cavity in the casting when cooled.

Each of the foregoing core binders possess disadvantages. For example, foundry pitch lacks "green strength" and is difficult to clean from the

5 cavities in the mold. Pulverized rosin solidifies upon storage, and cereal binders as heretofore produced lack adequate strength.

My invention is based upon the discovery that the foregoing difficulties and disadvantages may be substantially obviated by preparing a foundry core from core sand, a vehicle having binding properties such as molasses, or a drying or semi-drying vegetable oil such as linseed oil or soybean oil, water, and a corn flour which has been produced in a manner hereinafter to be described. My corn flour produces cores or molds possessing much greater strength than cores or molds employing cereal binders which have been processed according to the methods described in the prior art.

Accordingly one of the objects of my invention is the treatment of a ground degeminated corn product by a simple and inexpensive method whereby it will be adapted for use as a core binder.

A further object is to produce an improved high tensile strength sand core material such as is used in the casting of metals.

25 Another object of my invention is the production of a ground degeminated corn core binder having qualities superior to that of other corn product core binders.

Still another object is the development of a process which makes possible the use of a corn milling product which in normal times is a drug on the market. During the dry milling of degeminated corn a certain percentage of a more or less finely ground product is obtained, which 35 according to its degree of fineness, is known as corn flour or corn cream meal. That portion which passes through a 95 mesh screen is classified as a corn flour and the product which passes through a 46 mesh screen and is retained on a 40 95 mesh screen is commonly known as corn cream meal although sometimes broader ranges of particle size may be included under that terminology. My process enables the production of a valuable and efficient high quality core 45 binder from corn cream meal.

In practicing my invention, I have found that corn cream meal containing 10 to 15% moisture can be readily and economically pelleted. Any suitable means of pelleting may be employed, but I prefer to extrude the material through a die fitted with a revolving knife which is so adjusted that it cuts the pellets to an appropriate length. For ease of handling, I prefer pellets  $\frac{3}{8}$ " in diameter and  $\frac{1}{4}$ " in length. While the use of steam is not necessary in the extrusion

process, it is preferred since it apparently lubricates the dies, thus making for more efficient operation.

A charge of pellets produced as above described is placed in a puffing gun. This gun may be any of the conventional types of equipment used for the puffing of cereals such as rice, oats, wheat, corn, etc. Examples are the Anderson puffing gun such as that described in U. S. Patent 1,725,171 and the Plews puffing gun described in U. S. Patent 2,116,212. Superheated steam is allowed to enter the gun chamber at a temperature of 620° F. The steam passes through the pellets and expels any air present in the chamber. The cover of the puffing gun or chamber is then closed and the internal pressure allowed to build up to 175 lbs. per square inch. The chamber is maintained at this pressure for about three minutes whereupon the pressure is suddenly released. The resulting puffed corn cream meal cereal is then conveyed to a rotary drier and dried to a moisture content of about 8%. The dried material is then ground or pulverized to a flour of about 60 mesh. In the puffing process the temperature should be above the gelatinizing temperature of the starch in the cereal. A workable range is obtained by using superheated steam within a temperature range of 375° to 800° F. and a pressure range of 75 to 200 lbs. per square inch.

Cores manufactured from the above puffed pulverized corn cream meal are characterized by greater strength as indicated particularly by dry compression, air set compression and dry tensile strength tests. The following tests show the core binding qualities obtained with the puffed and then ground corn cream meal of the present invention as compared with flaked and pulverized corn products of the prior art.

A mixture of one part of puffed corn cream meal, 50 parts of sand and 1.5 parts of water was mixed for 8 minutes and produced a core which, when allowed to set in air for 30 minutes at room temperature, gave an air set compression of 16.8 lbs. per square inch and when baked for two hours at 400° F. gave a dry compression of 244 lbs. per square inch. When 30 parts of sand and 1 part of linseed oil were added to the above ingredients and another core formed and baked for one hour at 400° F., the resulting core had a tensile strength of 224 lbs. per square inch.

When a flaked and powdered mill starch product (unpuffed) was subjected to the same series of tests the air set compression was 8.8, the dry compression 100 and the dry tensile strength 140

lbs. per square inch. It is thus seen that the puffed corn cream meal product had a dry compression strength of twice that of the unpuffed product and an air set compression and dry tensile strength of somewhat less than double than that of the unpuffed product.

When a flaked and powdered product prepared from degemerinated corn grits (unpuffed) was subjected to similar sets of tests under identical conditions the dry compression, air set compression, and dry tensile strength was 115, 12.6 and 181 lbs. per square inch, respectively. Here, too, the puffed corn cream meal product is distinctly superior.

It is apparent from the above data that the puffed corn cream meal core binder is superior to both of the other corn product binders. In place of puffed corn cream meal one could use puffed corn flour and obtain similar advantageous results.

While I have in the above description disclosed what I believe to be a preferred and practical embodiment of my invention it will be understood that the specific details, including the technique by which the process is carried out, are by way of example and not to be construed as limiting the scope of the invention.

I claim:

1. A casting core material comprising a mixture of sand, a drying oil, and degemerinated, pelleted, puffed and pulverized corn flour.
2. A casting core material comprising a mixture of sand, a drying oil, and pulverized corn product formed by pelleting, steam puffing and comminuting a degemerinated, comminuted corn product.

JIM E. ALLISON.

#### REFERENCES CITED

40 The following references are of record in the file of this patent:

#### UNITED STATES PATENTS

| Number       | Name          | Date           |
|--------------|---------------|----------------|
| 45 707,892   | Anderson      | Aug. 26, 1902  |
| 921,030      | Wagner et al. | May 11, 1909   |
| 1,429,879    | Hill          | Sept. 19, 1922 |
| 2,181,372    | Kellogg       | Nov. 28, 1939  |
| 2,206,369    | Salzberg      | July 2, 1940   |
| 50 2,289,030 | Miller        | July 7, 1942   |
| 2,388,904    | Collatz       | Nov. 13, 1945  |

#### FOREIGN PATENTS

| Number     | Country       | Date         |
|------------|---------------|--------------|
| 55 515,470 | Great Britain | Dec. 6, 1939 |